# EUROPEAN PATENT SPECIFICATION

(11) **EP 3 390 908 B1**
(45) Date of publication and mention of the grant of the patent: **18.08.2021**
(21) Application number: 16874973.7
(22) Date of filing: 19.12.2016
(51) Int. Cl.: F23J 3/02, F28G 1/16, B24C 1/00, B24C 11/00

(54) **METHOD OF CLEANING HEAT TRANSFER SURFACES OF A POWERHOUSE**
VERFAHREN ZUR REINIGUNG VON WÄRMEÜBERTRAGUNGSFLÄCHEN EINES MASCHINENHAUSES
PROCÉDÉ DE NETTOYAGE DE SURFACES DE TRANSFERT DE CHALEUR D'UNE SALLE DES MACHINES

(30) Priority: 18.12.2015 FI 20155970
(43) Date of publication of application: 24.10.2018
(73) Proprietor: Clean Steel International Oy, 28600 Pori (FI)
(72) Inventor: LAITOMAA, Hannu, 28400 Ulvila (FI); LAITOMAA, Juuso, 28400 Ulvila (FI); LAITOMAA, Janne, 28400 Ulvila (FI)
(74) Representative: Laine IP Oy
(86) International application number: PCT/FI2016/050897
(87) International publication number: WO 2017/103345

(56) References cited:
- EP-A1- 2 113 339
- EP-A1- 2 113 339
- WO-A1-94/08755
- DE-A1- 19 723 389
- DE-A1- 19 723 389
- US-A- 4 348 340
- US-A- 4 348 340
- US-A- 4 666 083

## Description

The present invention relates to a method according to the preamble of claim 1 of cleaning the heat-transfer surface which is in connection to the masonry structure of a combustion boiler. Such a method is disclosed in DE 197 23 389.

In such a method, the surface is cleaned by blasting solid particles onto it.

The heat-transfer surfaces of power plants are typically cleaned by using sandblasting. In this case, sand (typically screened sand) is used in the sandblasting, and water is used to bind the fines, in order to prevent dusting caused by the sand particles. This wet blasting method has proven to be problematic in several respects.

When burning wood or fossil fuels, also sulphur and organic compounds which are derived from the combustion, are generated in the boiler. By providing water to the ashes which remain on the fire surfaces, various acids and weak acids start to form in the boiler. However, it is not possible to clean the boiler completely with water. Instead, the residual ash remains wet and acidic. The acids and the weak acids begin to corrode the steel. Moisture can also reach the inner part and the gaps of the masonry, and at same time, cause corrosion.

When damp ash dries, it becomes almost as hard as concrete. Repeated washes with water gradually accumulate more and more hard surface in the pipes, which reduces the efficiency of the heat production and reduces the flow of gases. Removing the hardened ash from inside the eco- and the superheater packages is very difficult and laborious, in some structural solutions even impossible and, as a result, the only possibility may be to replace part of or all of the structure.

It should also be noted that the masonries absorb moisture. The heating phase of the start-up stage is extended because the masonries must be "dried". In such cases, it is quite possible that the masonries will fail.

In the prior art, various alternatives are described for using sand in the blasting. Such materials include steel grains and steel sand, copper slag, glass beads, metal pellets, dry ice, corundum and even ground coconut shells and corn grains.

CN Patent Application Publication No. 102313288 describes a solution in which heat-transfer surfaces are cleaned using smooth-surface particles. In particular, the particles described in the publication are metal or non-metal particles or composite particles having a density of 2-8 g/cm³.

DE Patent Application Publication No. 19723389 describes cleaning of the inner part of the boiler plants where the combustion gases are by using spherical steel particles.

International Application Publication WO 0138815 suggests blast cleaning of the heat-transfer surfaces by using coarse ash which is generated from the incineration of sludge.

JP Patent Application Publication No. 2002098323 describes the use of granulated slag grains to remove, by using blast cleaning, the metal residues which are adhered to the exhaust pipe of an electric furnace. The metal is generated when melting, in an electric furnace, the burning residues which are generated from burning of municipal waste.

Furthermore, the known technology is disclosed in US Patent Specifications Nos. 4 348 340 and 4 666 083.

Also previously known are dry blasting methods. An example of such a method is the solution which is described in the EP Patent Application Publication No. 2 113 339, in which alkali metal carbonates are used for blast cleaning of solid surfaces. According to the publication, alkali metal carbonates provide efficient cleaning of surfaces, without formation of dust or damaging the surfaces. Suitable materials mentioned in the publication are in particular natural carbonates, such as calcium carbonate and dolomite. These may be used, for example, to remove paint, foodstuff and drug residues from the inner

As described above, to date, no solutions have been proposed with which it would be possible to remove stubborn deposits, which are generated at temperatures that are typical for combustion boilers, without damaging the surfaces and without the formation of dust, which is characteristic of sand.

In the present invention, we have unexpectedly discovered that the above objective can be achieved by using, for the blasting, nickel slag particles in essentially dry conditions.

Thus, according to the present invention, the heat-transfer surface of the combustion boiler, especially the heat-transfer surface which is in connection to a masonry structure, is cleaned by blasting onto it, in water-free conditions, metal slag particles having a particle size of approximately 0.3 - 2.5 mm, and by using a blasting pressure of 8-12 bar.

Thus, the present invention also comprises the use of nickel slag particles for cleaning of the heat-transfer surface which is in connection to a masonry structure, by using blasting treatment.

More specifically, the method according to the present invention is mainly characterised by what is stated in the preamble of Claim 1.

Considerable advantages are achieved with the present invention. By replacing sand in the blasting cleaning with nickel slag particles in dry conditions, it is possible to remove the dirt on the metal surface in objects which are difficult to clean without damaging the surface. At the same time, it is possible to avoid the damaging effect of the water flowing from the surface to be cleaned onto the masonry structures which are in contact with the surface or are near the surface.

Furthermore, it has been found that dusting is considerably lower than in sandblasting, even though the operation is carried out in water-free conditions, which contributes to the work performance.

The slag particles, which represent the waste fraction, and which otherwise cannot be used in any significant application, form an economically and technically advantageous material which, if needed, can be ground and graded in order to achieve a fraction of a desired fineness.

The nickel slag particles are particularly well suited for the cleaning of steel heat-transfer surfaces, because the nickel slag do not comprise significant amounts of ferrite compounds. This, in turn, means that when cleaning steel surfaces with nickel slag, no corrosion problems appear, which is not the case when blasting with metal slags that comprise ferrite compounds, or when blasting with for example steel particles that also comprise ferrite compounds.

In the following, embodiments will be examined more closely with the aid of the accompanying detailed description.

In the application of the present technology, heat-transfer surfaces of a power plant, in dry conditions, are cleaned using a fine fraction of a waste product generated in a metallurgical process. In one embodiment, especially the heat-transfer surfaces that are connected to the structures of a combustion boiler, in particular the masonry structures of a combustion boiler, are cleaned.

Typically, the surface to be cleaned comprises sulphur or silicate-bearing compounds which are generated when burning wood or fossil fuels or mixtures thereof, and possibly ash, coke or slag which comprise organic compounds (such as tar-like compounds).

Especially, in an embodiment, deposits and similar dirt layers which are generated during the combustion process are removed from the metal surfaces without substantially damaging these.

In the present technology, the operation is carried out in essentially "water-free conditions". In practice, this means that water or aqueous solutions are not fed, either together with or separately from the blasted particles, onto the object to be cleaned. Typically, no water or aqueous solutions at all are fed. However, if together with the particles, moisture ends up in the object to be cleaned, operating in water-free conditions means that, due to the effect of particle blasting, condensed water does not flow from the surface to be cleaned into the adjacent structure, which, for example, is masonry.

Typically, the surface to be cleaned is a heat-transfer surface. However, the method can also be used to clean other surfaces of a power plant boiler structure, which surfaces comprise impurities, including ash, coke and/or slag deposits which are generated from the combustion.

In one embodiment, the structure to be cleaned is part of a power boiler, such as a heat boiler, or part of a recovery boiler, such as a kiln for reburning lime sludge or a soda recovery unit.

The heat-transfer surface is a metal surface, typically it is a steel surface. The steel may be, for example, a ferritic or an austenitic steel alloy which meets ASTM standards A213 or A213M, respectively. It is also possible to use other types of metal alloys. However, the surfaces may be of a material other than metal, for example a ceramic.

Examples of surfaces to be cleaned are, in particular, the heat-transfer surface which forms part of a heat boiler, such as the eco- and the superheater packages of grate-fired boilers or fluidised bed boilers.

In one embodiment, the surface to be cleaned, a metal surface, typically a steel surface, forms at least part of a superheater or at least part of an Economizer or a Luvo unit.

Preferably, the surface to be cleaned is in the vicinity of the masonry or at least partly on top of it. Typically, the distance to the nearest masonry, i.e. the masonry surface, is at maximum approximately 250 cm, usually at maximum approximately 150 cm, especially at maximum approximately 100 cm, for example at maximum 50 cm. The masonry surface may be in direct contact with the surface to be cleaned.

It is well known that those parts of the wall structures of boilers that are designed for burning moist fuels, and which parts maintain a temperature suitable for the drying and the pyrolysis phases, should be uncooled. An uncooled surface is achieved, for example, by using masonries. For example, ceramic bricks can be used for the masonry. At the fuel layer points, in turn, the furnace walls are cooled, which can reduce the problems that arise when the fuel burns too quickly at the edges of the grate.

According to the invention, the blasting is carried out with nickel slag, which is in particle form, in which case the particle size of the nickel slag is approximately 0.3-2.5 mm.

Here, "nickel slag" means the by-product which is generated in the production or cleaning of the metal in question, i.e. in general "material", which typically is primarily silicate-based. The silicate material is, nickel silicate, and it comprises, besides the main component, also for example metals which are derived from the metal raw material, and alkaline earth metals, and their compounds, such as oxides, sulphates, sulphides and silicates.

According to a preferred embodiment, nickel slag is used which is essentially free of ferritic compounds.

According to a preferred embodiment, nickel slag is used, the particles of which are non-spherical shaped.

According to the invention, nickel slag is used. This is a waste product which is generated in association with the recovering of nickel.

Experiments have demonstrated that the particle material of the nickel slag used must have, besides a particle size which is suitable for the blasting, also a sufficient hardness and weight. Typically, the hardness of the nickel slag particles must be greater than approximately 6°, most suitably even approximately 8°, on the Mohs scale of hardness, and the density must be greater than approximately 3.0 g/cm³, for example approximately 3.1-4.2 g/cm³, most suitably approximately 3.3-3.9 g/cm³, or 3.5-3.8 g/cm³. The hardness can be over 8° on the Mohs scale, but usually a hardness of approximately 8° (± 0.5°) is sufficient to carry out the cleaning.

Besides a sufficient specific gravity, the particles must have a suitable shape. Thus, the bulk density is greater than 1.8 g/cm³, especially 1.85 g/cm³ or greater.

When the hardness, shape, and weight of the material used are within the ranges described above, the dirt can be removed from the object to be cleaned. With excessively light or chip-like slag, the result will not be as desired.

In addition, in preferred applications, the particle size of the slag is within a pre-selected range.

The present particles may be individual particles or agglomerates (granules) which are formed of several particles.

According to the invention, the average particle size of the nickel slag is within the range of 0.3-2.5 mm, for example 0.5-2.2 mm. Typically, this means that the maximum dimension of least 90 % of the particles, most suitably at least approximately 95 % (by weight) is within the said range.

Here, the particle size typically means the screened particle size (that is, grain-size).

It has been found that, with a narrow distribution of particle size, in which at least 90 %, especially at least 95 % of the particles (by weight) have the particle size defined above, in particular with regard to the largest dimension, it is possible to maintain a predetermined pressure in the blasting stream, in which case a uniform effect over the surface is obtained. Typically, the pressure range is 8-12 bar, see below.

It has been discovered that the nickel slag particles are not spherical, but they have an irregular shape. This also means that, when the blasted nickel slag particles hit the surface, both the surface pressure generated and the interaction between the particles and the surface are different from the case where spherical particles are used. The width of the contact area of individual slag particles varies depending on which part of the particle hits the surface. Thus, by using slag particles, the ash layer remaining on the surface can be loosened more efficiently than with steel balls, without damaging the steel surface.

In the present invention, typically the blast nozzle used can be either small or large. The nozzle diameter may be, for example, 0.5-25 mm, usually approximately 1-15 mm, typically approximately 12 mm. These nozzle sizes are particularly suitable for the application described above, in which the nickel slag particles have a narrow distribution of particle size.

The blasting is carried out by using a blasting pressure of 8-12 bar. More preferably, the pressure used is 9-11 bar. At this pressure, an efficient cleaning of the dirt layers is achieved and, at the same time, damage to the surface is avoided. The consumption of air varies with the nozzle size, but is generally approximately 50-2500 1/min, most suitably approximately 70-1500 1/min, for example approximately 150-1000 1/min.

The blasting can be carried out by using a nozzle which is straight, curved or bent at 45 degrees. The shape of the nozzle is selected according to the object to be cleaned.

In connection with the present invention, we have found that after cleaning carried out using the slag particles described, the surface does not corrode as easily as after treatment in which sand is used. In addition, after the present treatment, the surface is not prone to become dirty. One of the reasons for this seems to be that for example nickel slag forms a chromium oxide compound on the metal surface, which compound protects the metal from corrosion, and which, on the other hand, also slows down the adhesion of new dirt to the metal surface.

### Citation List

Patent literature
CN 102313288
DE 19723389
WO 0138815
JP 2002098323
EP 2 113 339
US 4 348 340
US 4 666 083

## Claims

1. A method of cleaning a heat-transfer surface connected to a masonry structure of a combustion boiler, in which method the surface is cleaned by blasting solid particles onto it, in essentially water-free conditions, **characterised in that** a metal surface, in particular steel surface, is cleaned,_the blasting is carried out at a pressure of 8-12 bar, using particles of nickel slag, with
- a hardness of greater than 6° on the Mohs scale of hardness, especially greater than 6° and at maximum approximately 8° on the Mohs scale,
- a density of 3.1-4.2 g/cm³, most suitably 3.3-3.9 g/cm³, for example 3.5-3.8 g/cm³,
- a bulk density which is greater than 1.8 g/cm³, especially 1.85 g/cm³ or greater, and
- the particle size used is 0.3-2.5 mm.

2. A method according to Claim 1, **characterised in that** the heat-transfer surface to be cleaned forms part of the surface of a heat exchanger of a boiler, forms at least part of a superheater or forms at least part of an Economizer or a Luvo unit.

3. A method according to any of the preceding claims, **characterised in that** the surface to be cleaned comprises ash that includes sulphur or organic compounds which are generated when wood or fossil fuels have been burned.

4. A method according to any of the preceding claims, **characterised in that** a nickel slag is used, which is essentially free from ferritic compounds.

5. A method according to any of the preceding claims, **characterised in that** a nickel slag is used, the particles of which are non-spherical shaped.

6. A method according to any of the preceding claims, **characterised in that** the pressure used is 9-11 bar.

7. A method according to any of the preceding claims, **characterised in that** the blasting is carried out using a 12 mm nozzle, which is straight, curved or bent at 45 degrees.

8. A method according to any of the preceding claims, **characterised in that** the structure to be cleaned is part of a power boiler, such as a heat boiler, or part of a recovery boiler, such as a kiln for reburning lime sludge or a soda recovery unit.

9. A method according to any of the preceding claims, **characterised in that** the surface to be cleaned is in the vicinity of the masonry or at least partly on top of it.

10. A method according to any of the preceding claims, **characterised in that** particles of nickel slag are used, which have a narrow distribution of particle size, in order to achieve a uniform effect over the surface to be cleaned, the pressure being 8-12 bar in the stream used in the blasting .

11. The method according to Claim 10, **characterised in that** the blasting is carried out using a nozzle, the diameter of which is 0.5-25 mm, generally approximately 1-15 mm, especially approximately 12 mm.

## Patentansprüche

1. Verfahren zum Reinigen einer Wärmeübertragungsfläche, die mit einem Mauerwerk eines Verbrennungskessels verbunden ist, bei welchem Verfahren die Oberfläche durch Strahlen fester Teilchen auf sie unter im Wesentlichen wasserfreien Bedingungen gereinigt wird,
**dadurch gekennzeichnet, dass** eine Metallfläche, insbesondere Stahlfläche, gereinigt wird, wobei das Strahlen bei einem Druck von 8-12 bar unter Verwendung von Teilchen einer Nickelschlacke ausgeführt wird, mit
- einer Härte von mehr als 6° auf der Mohsschen Härteskala, insbesondere größer als 6° und bei maximal etwa 8° auf der Mohsschen Härteskala,
- einer Dichte von 3,1-4,2 g/cm³, am geeignetsten 3,3-3,9 g/cm³, zum Beispiel 3,5-3,8 g/cm³,
- einer Schüttdichte, die größer als 1,8 g/cm³, insbesondere 1,85 g/cm³ oder mehr ist und
- die verwendete Teilchengröße 0,3-2,5 mm ist.

2. Verfahren nach Anspruch 1, **dadurch gekennzeichnet, dass** die zu reinigende Wärmeübertragungsfläche Teil der Oberfläche eines Wärmetauschers eines Kessels bildet, mindestens Teil eines Überhitzers bildet oder mindestens Teil einer Economizer- oder einer Luvo-Einheit bildet.

3. Verfahren nach einem der vorstehenden Ansprüche, **dadurch gekennzeichnet, dass** die zu reinigende Oberfläche Asche umfasst, die Schwefel oder organische Verbindungen beinhaltet, die erzeugt werden, wenn Holz oder fossile Brennstoffe verbrannt werden.

4. Verfahren nach einem der vorstehenden Ansprüche, **dadurch gekennzeichnet, dass** eine Nickelschlacke verwendet wird, die im Wesentlichen frei von ferritischen Verbindungen ist.

5. Verfahren nach einem der vorstehenden Ansprüche, **dadurch gekennzeichnet, dass** eine Nickelschlacke verwendet wird, deren Teilchen nicht kugelförmig geformt sind.

6. Verfahren nach einem der vorstehenden Ansprüche, **dadurch gekennzeichnet, dass** der verwendete Druck 9-11 bar ist.

7. Verfahren nach einem der vorstehenden Ansprüche, **dadurch gekennzeichnet, dass** das Strahlen unter Verwendung einer 12 mm Düse ausgeführt wird, die gerade, gekrümmt oder bei 45 Grad gebogen ist.

8. Verfahren nach einem der vorstehenden Ansprüche, **dadurch gekennzeichnet, dass** die zu reinigende Struktur Teil einer Kesselanlage ist, wie eines Heizkessels, oder Teil eines Rückgewinnungskessels, wie eines Ofens zum Rekalzinieren von Kalkschlamm oder eine Sodarückgewinnungseinheit.

9. Verfahren nach einem der vorstehenden Ansprüche, **dadurch gekennzeichnet, dass** die zu reinigende Oberfläche in der Nähe des Mauerwerks oder zumindest teilweise auf dessen Oberseite ist.

10. Verfahren nach einem der vorstehenden Ansprüche, **dadurch gekennzeichnet, dass** Teilchen von Nickelschlacke verwendet werden, die eine enge Verteilung von Teilchengröße aufweisen, um eine gleichförmige Wirkung über die zu reinigende Oberfläche zu erzielen, wobei der Druck 8-12 bar in dem Strom ist, der zum Strahlen verwendet wird.

11. Verfahren nach Anspruch 10, **dadurch gekennzeichnet, dass** das Strahlen unter Verwendung einer Düse ausgeführt wird, deren Durchmesser 0,5-25 mm, im Allgemeinen etwa 1-15 mm, insbesondere etwa 12 mm ist.

## Revendications

1. Procédé de nettoyage d'une surface de transfert de chaleur reliée à une structure de maçonnerie d'une chaudière à combustion, procédé dans lequel la surface est nettoyée par décapage au moyen de particules solides, dans des conditions essentiellement sans eau,
**caractérisé en ce qu'**une surface de métal, en particulier une surface d'acier, est nettoyée, le décapage est effectué à une pression de 8 à 12 bars, en utilisant des particules de scorie de nickel, avec
- une dureté supérieure à 6° sur l'échelle de dureté de Mohs, particulièrement supérieure à 6° et au maximum d'environ 8° sur l'échelle de Mohs,
- une densité de 3,1 à 4,2 g/cm³, de façon la plus appropriée de 3,3 à 3,9 g/cm³, par exemple 3,5 à 3,8 g/cm³,
- une densité apparente qui est supérieure à 1,8 g/cm³, particulièrement 1,85 g/cm³ ou plus, et
- la taille de particule utilisée est de 0,3 à 2,5 mm.

2. Procédé selon la revendication 1, **caractérisé en ce que** la surface de transfert de chaleur à nettoyer forme une partie de la surface d'un échangeur de chaleur d'une chaudière, forme au moins une partie d'un surchauffeur ou forme au moins une partie d'un Économiseur ou d'une unité Luvo.

3. Procédé selon l'une quelconque des revendications précédentes, **caractérisé en ce que** la surface à nettoyer comprend des cendres qui incluent des composés organiques ou soufrés qui sont produits quand du bois ou des combustibles fossiles ont été brûlés.

4. Procédé selon l'une quelconque des revendications précédentes, **caractérisé en ce que** des scories de nickel sont utilisées, qui sont essentiellement exemptes de composés ferritiques.

5. Procédé selon l'une quelconque des revendications précédentes, **caractérisé en ce que** des scories de nickel sont utilisées, dont les particules sont de forme non sphérique.

6. Procédé selon l'une quelconque des revendications précédentes, **caractérisé en ce que** la pression utilisée est de 9 à 11 bars.

7. Procédé selon l'une quelconque des revendications précédentes, **caractérisé en ce que** le décapage est effectué en utilisant une buse de 12 mm, qui est droite, courbe ou pliée à 45 degrés.

8. Procédé selon l'une quelconque des revendications précédentes, **caractérisé en ce que** la structure à nettoyer fait partie d'une chaudière de production d'énergie, comme une chaudière de production de chaleur, ou une partie d'une chaudière à récupération, comme un four pour rebrûler les boues de chaux ou une unité de récupération de soude.

9. Procédé selon l'une quelconque des revendications précédentes, **caractérisé en ce que** la surface à nettoyer est au voisinage de la maçonnerie ou au moins en partie sur le dessus de celle-ci.

10. Procédé selon l'une quelconque des revendications précédentes, **caractérisé en ce que** des particules de scories de nickel sont utilisées, qui présentent une distribution étroite de taille de particule, afin de parvenir à un effet uniforme sur la surface à nettoyer, la pression étant de 8 à 12 bars dans le flot utilisé lors du décapage.

11. Procédé selon la revendication 10, **caractérisé en ce que** le décapage est effectué en utilisant une buse, dont le diamètre est de 0,5 à 25 mm, de manière générale d'environ 1 à 15 mm, particulièrement environ 12 mm.
